

[54] LEACHING AGGLOMERATED GOLD -  
SILVER ORES

[75] Inventors: Harold J. Heinen, Reno; Gene E. McClelland, Sparks; Roald E. Lindstrom, Reno, all of Nev.

[73] Assignee: The United States of America as represented by the Secretary of the Interior, Washington, D.C.

[21] Appl. No.: 141,088

[22] Filed: Apr. 17, 1980

#### Related U.S. Application Data

[63] Continuation-in-part of Ser. No. 29,952, Apr. 13, 1979, abandoned, and Ser. No. 29,953, Apr. 13, 1979, abandoned.

[51] Int. Cl.<sup>3</sup> ..... C01G 5/00; C01G 7/00

[52] U.S. Cl. ..... 423/29; 75/3;  
75/105; 75/118 R

[58] Field of Search ..... 423/27, 29; 75/101 R,  
75/105, 106, 118, 3

#### [56] References Cited

##### U.S. PATENT DOCUMENTS

|           |         |                |        |
|-----------|---------|----------------|--------|
| 588,476   | 8/1897  | Rhodes .....   | 423/27 |
| 658,938   | 10/1900 | Alzugary ..... | 75/105 |
| 868,551   | 10/1907 | Hall .....     | 75/105 |
| 2,009,667 | 7/1935  | Keyes .....    | 423/29 |

##### FOREIGN PATENT DOCUMENTS

|        |        |                      |      |
|--------|--------|----------------------|------|
| 517867 | 2/1940 | United Kingdom ..... | 75/3 |
|--------|--------|----------------------|------|

##### OTHER PUBLICATIONS

*Chemical Abstracts*, vol. 68, No. 97,730c (1968).

Primary Examiner—Brian E. Hearn  
Attorney, Agent, or Firm—William S. Brown; Donald A. Gardiner

#### [57] ABSTRACT

Percolation leaching of gold or silver ores, tailings or wastes is accomplished by a process comprising initial agglomeration of fines in the feed by means of a binding agent and cyanide solution, followed by aging and, subsequently, leaching to recover gold or silver values.

7 Claims, No Drawings

## LEACHING AGGLOMERATED GOLD - SILVER ORES

This application is a continuation-in-part of applications Ser. Nos. 29,952 and 29,953, filed Apr. 13, 1979, both abandoned.

Conventional percolation leaching, particularly heap leaching, has generally proven to be a low-capital, low-operating cost technique for processing low-grade gold or silver ores, tailings or wastes. However, many such materials are not amenable to existing percolation leaching processes because of the presence of excessive amounts of clays, or of fines generated during crushing of the feed materials. These constituents in the feed 10 impede uniform flow of leach solution through the feed beds, causing channeling and reducing precious metal recovery. In the mineral processing field, slimes are generally defined as the fraction of an ore that is too fine to be commercially exploited by processes developed for the coarser size fractions. Frequently slimes are 15 considered to be particles less than 50 microns in diameter. Slimes are present in most ores and mill feeds because of (1) weathering, physical abrasion, and alterations of certain rock components, and (2) the comminution of the ore to achieve liberation of the valuable mineral constituents. In prevailing heap leach cyanidation practices, the presence of slimes (clays and/or ore fines) in the feed materials impede uniform solution 20 flow through the ore mass and channeling results which reduces precious metal extraction. In extreme cases, the presence of clays can completely seal the ore heap causing the leach solution to run off the sides of the heap rather than penetrate the ore. Because prevailing technology is inadequate to handle the slime problem in 25 heap leach cyanidation, many of the low-grade clayey gold and silver deposits cannot be exploited.

It was found, in accordance with the process of application Ser. No. 29,953, that the efficiency of percolation leaching processes for recovery of gold or silver from such feed materials could be substantially improved by 30 initial pretreatment of the feed with a binding agent and water to agglomerate fines contained in the feed, followed by aging of the thus-treated feed. The pretreated feed could then be subjected to conventional percolation leaching techniques to recover gold or silver values.

It was also found, in accordance with the process of application Ser. No. 29,952, that the speed and efficiency of such percolation leaching processes could be substantially improved by initially wetting the feed with a relatively concentrated alkaline cyanide solution, allowing the wetted feed to age for a time sufficient for substantially complete reaction with gold or silver values in the feed, and then leaching soluble gold or silver 45 cyanides from the aged feed with water.

It has now been found, according to the process of the present invention, that the efficiency of percolation leaching processes for recovery of gold or silver from such feed materials may be still further improved by initial pretreatment of the feed with a binding agent and an aqueous cyanide solution to agglomerate the fines contained in the feed, as well forming soluble cyanides of gold or silver values in the feed. The method of the invention consists of wetting the crushed ore, or other finely divided feed material, with an alkaline cyanide solution considerably more concentrated than that conventionally employed, allowing the wetted ore to age

for a time sufficient for agglomeration of fines in the ore and for substantially complete reaction of the cyanide with gold or silver, and then leaching soluble gold or silver cyanides from the aged ore. Essentially all of the leachable precious metal content of the ore is removed in about ten hours or less, the free cyanide and alkali content of the leach solution is very low, and the residual cyanide in the spent ore is generally only a fraction of a part per million.

Although a fairly concentrated cyanide solution is used to pretreat the ore, the ore takes up only enough cyanide to react with its precious metal content, thereby reducing total cyanide consumption as compared to conventional practice. In some cases it is not even necessary to add protective alkali to the cyanide solution, hydrolysis of the sodium cyanide being sufficient to raise the pH to the proper level.

More specifically, the invention relates to a process involving the steps of (1) mixing the feed with a binding agent, (2) wetting the feed-binding agent mixture uniformly with a closely controlled amount of cyanide solution, (3) mechanically manipulating the wetted material to effect agglomeration of fines contained in the feed, (4) aging the thus-treated feed at ambient conditions until the agglomerates have set up and developed sufficient green strength to withstand further wetting without disintegration, and the reaction of the cyanide with gold or silver values is substantially complete, and (5) subjecting the pretreated feed to conventional percolation leaching for extraction of gold or silver values. This pretreatment of the feed increases its porosity and permeability, thus enhancing the percolation flow of leach solutions through beds or heaps of the gold or silver-containing feed. Both the speed and extraction efficiency of the leaching process is thereby substantially improved. In addition, the amount of residual leach solution, specifically cyanide, in the spent feed is reduced, and the resulting pregnant leach solutions are lower in free cyanide and alkalinity, thereby facilitating recovery of gold and silver values by carbon adsorption.

Burnt lime, i.e., calcium oxide, and type II portland cement have been found to be particularly effective as binding agents in the process of the invention. However, other binding agents, such as calcium aluminate cement, magnesia, dolomite, inorganic silicates and organic long chained polymers, may also be used. In addition, other types of lime, such as hydrated and agricultural lime, and other varieties of portland cement may also be used as the binding agent. Particular combinations of these binding agents may also be effective for treatment of specific feed materials.

Flocculating agents, including lime, have been widely employed in thickening and dewatering applications, such as dewatering ore pulps, and briquetting or pelletizing finely ground concentrates into larger particles suitable for heat hardening prior to charging to an open hearth or blast furnace. The primary purpose of such procedures is production of briquettes or pellets that do not spall during thermal induration. In contrast, the objective of applicants' invention was conversion of fines in feed materials to porous agglomerates having sufficient green strength to withstand percolation leaching, as well as rapid and efficient formation of soluble cyanides of gold and silver values. Lime is also frequently used to provide protective alkalinity in conventional cyanide heap leaching. However, its use in this

manner has little beneficial effect on the percolation flow through ore beds.

In the process of the invention, the feed is thoroughly mixed with a small amount of the binding agent, and the mixture is then wetted with an amount of cyanide solution sufficient to cause substantial binding or agglomeration of fines in the feed, and to form soluble cyanides with a major portion of the gold or silver values when the mixture is cured or aged for a suitable period of time. Optimum amounts of binding agent and cyanide solution will vary with the type of feed and specific binding agent and cyanide solution employed. However, suitable amounts of binding agent will usually be in the range of about 5 to 15 pounds per ton of feed, with the amount of cyanide solution generally being in the range of about 8 to 16 weight percent based on the amount of feed. Close control of the amount of cyanide solution has, however, been found to be generally desirable since best results are usually obtained only when a particular amount of solution is used in the agglomeration process. This will generally be an amount sufficient to uniformly wet or dampen, but not necessarily inundate, the ore particles. Since, however, the optimum amount of solution may vary considerably with different feed materials and binding agents, this amount is best determined experimentally. By proper control of the quantity of binding agent and solution, only the fines are agglomerated, leaving the coarser fragments of the feed material relatively unaffected. This results in a granular, popcorn-like product of substantially increased porosity and permeability.

The cyanide solution will generally consist of aqueous sodium cyanide, although solutions of calcium or potassium cyanide may also be employed. Optimum concentration of the cyanide solution may vary considerably depending on the specific type and amount of ore, although, as discussed above, a relatively concentrated solution is employed. Concentrations of sodium cyanide of about 5 to 20 lbs per ton of solution are generally satisfactory. Sodium hydroxide, lime or sodium carbonate is employed in the cyanide solution in an amount sufficient to provide protective alkalinity as in conventional cyanide leaching practices. Generally, an amount sufficient to provide pH of about 10 to 11 is satisfactory, although in some cases the hydrolysis of the sodium cyanide will maintain optimum alkalinity without addition of alkali.

The cyanide solution may be added and admixed with the feed-binding agent mixture by any conventional means such as a pelletizer or balling machine. Agglomeration of fines in the resulting admixture is also accomplished by conventional mechanical means such as the use of a rotating disk pelletizer or balling machine to produce agglomerates, pellets or balls from the fines. Generally, admixture of the feed-binding agent mixture with the solution, and agglomeration, may be effected simultaneously by means of such mechanical devices. Although this procedure for preparation of the wetted feed-binding agent mixture is generally preferred, other methods, such as spraying a slurry of the binding agent onto the dry feed, may also be used.

The resulting material is then aged or cured, without drying, at ambient conditions for a period of time sufficient to cause the agglomerates to set up and develop sufficient green strength to withstand further wetting without disintegration, as well as effecting reaction of the cyanide solution with gold or silver values. Although optimum aging time may also vary considerably

with specific feed material and binding agent, suitable times will usually fall within the range of about 5 to 72 hours. Use of appropriate accelerators, particularly where the binding agent is cement, may, however, reduce the required aging considerably. Again, however, the time of aging has been found to be important to achievement of best results and optimum aging time should, therefore, be determined experimentally in each case.

Leaching of the thus-pretreated feed to extract gold or silver values is accomplished by conventional percolation leaching procedures, such as heap leaching or vat leaching. Such procedures consist of percolation of leach solution through a body of the feed material in order to extract gold or silver values in the form of cyanide complexes of the metals. Details of such procedures are well known in the art and do not constitute an essential aspect of the invention. A detailed description of heap leaching of gold ores, e.g., is given in Bureau of Mines Information Circular 8770, 1978.

The leach solution may consist of water or a dilute cyanide solution, preferably sodium cyanide solution of a concentration of about 0.1 to 0.5 lb/ton of solution. It has been found, however, in accordance with a preferred embodiment of the invention, that the process is generally most efficiently carried out by means of initial leaching with water, followed by recovery of the gold or silver values by conventional means, e.g., by adsorption on activated carbon, and recycle of the leach solution for further leaching of the pretreated feed. Since the leaching procedure results in accumulation of small concentrations of cyanide in the aqueous leachant, the leach solution in subsequent leaching steps will consist of a dilute cyanide solution. Generally, the leach solution may be recycled throughout the leaching period without substantial decrease in leaching efficiency. The invention, and the advantages thereof, will now be more specifically illustrated by the following examples. The percolation leach tests of these examples were conducted on 50-lb charges of feed material in a plexiglass column 5 feet high with an inside diameter of 5.5 inches to make a bed about 4 feet in height. Twelve liters of leach solution, either water or dilute cyanide solution, was employed. After bedding the feed materials in the leach column, downward directed percolation leaching was initiated. The pregnant liquor was collected in a sump, pumped upward through activated carbon for silver-gold recovery and the resulting barren solution was returned to the top of the leach column. The leach solution was recirculated through the leaching-carbon adsorption system until a steady-state flow rate had been achieved. Flow rate measurements were taken daily for a period of one week, and averaged to determine the percolation flow rate.

#### Example 1

In this example, two gold ore samples from the same property were employed in leaching experiments. The first sample was a surface material containing 0.1 oz Au/ton and only small amounts of clayey and fine material. The second sample was from 45-90 feet below the surface and contained 0.2 oz Au/ton of ore and significant amounts of clayey and fine material. A series of three column leach test using 50 lbs of ore crushed to a nominal  $\frac{1}{2}$  inch feed size were conducted on each of the two samples. The three tests consisted of: (1) a baseline test with no pretreatment (conventional percolation leach), (2) a test employing agglomeration of fines in the

feed with a combination of type II portland cement, in an amount of 10 lbs/ton of feed, and water, in amount of 7.7-12 weight percent based on the amount of feed, and (3) a test employing agglomeration of fines in the feed and formation of soluble gold cyanide by means of a combination of the same amount of type II portland cement and an aqueous sodium cyanide, containing 8.7-13.5 lb NaCN/ton of solution, the amount of solution being 7.7-12 weight percent based on the amount of feed.

Results of these tests are shown in Table 1. The data indicate that agglomeration of fines of the surface material was not essential for an adequate percolation rate (9.1 gal/hr/ft<sup>2</sup>), although particle agglomeration with portland cement and either water or cyanide solution

ducted in essentially the same manner as the leaching experiments of example 1. Results are shown in Table 2. The data indicate that agglomeration of fines with portland cement and water was effective in improving percolation rate and substantially reducing leaching time for maximum silver recovery as compared to conventional heap leaching techniques. Cyanide consumption was also reduced by 33 percent.

Pretreatment with a combination of portland cement and cyanide solution was also effective in improving percolation rates and reducing cyanide consumption, but was even more effective in reducing the leaching time (2.3 days vs 22 days for no pretreatment and 11 days for pretreatment with the combination of cement and water).

TABLE 1

| Sample     | Pretreatment                                          | Pertinent column leach data from six percolation leach experiments |                    |                               |                  |                                          |                       |     | CN <sup>-</sup> cons, lb/ton ore | Au recovery, pct total Au |
|------------|-------------------------------------------------------|--------------------------------------------------------------------|--------------------|-------------------------------|------------------|------------------------------------------|-----------------------|-----|----------------------------------|---------------------------|
|            |                                                       | Experimental calculated head, oz Au/ton ore                        | Cement, lb/ton ore | Reagents Cyanide, lb/ton soln | Moisture, wt-pct | Percolation rate, gal/hr/ft <sup>2</sup> | Leaching period, days |     |                                  |                           |
| Surface    | None                                                  | 0.10                                                               | —                  | 2                             | —                | 9.1                                      | 5                     | 0.4 | 90.1                             |                           |
|            | Particle agglomeration with cement + H <sub>2</sub> O | .11                                                                | 10                 | 2                             | 7.7              | 19.2                                     | 5                     | .4  | 90.9                             |                           |
|            | Particle agglomeration with cement + CN               | .11                                                                | 10                 | 13.5*                         | 7.7              | 21.1                                     | 1.5                   | .3  | 91.0                             |                           |
| Clayey ore | None                                                  | .21                                                                | —                  | 2                             | —                | .5                                       | 9                     | .4  | 90.6                             |                           |
|            | Particle agglomeration with cement + H <sub>2</sub> O | .23                                                                | 10                 | 2                             | 12.0             | 19.7                                     | 5                     | .4  | 91.2                             |                           |
|            | Particle agglomeration with cement + CN               | .23                                                                | 10                 | 8.7*                          | 12.0             | 19.5                                     | 2                     | .3  | 91.4                             |                           |

\*based on cyanide content of the pretreatment solution.

TABLE 2

| Sample            | Pretreatment                                          | Pertinent column leach data from three percolation leach experiments on a high clay containing silver ore |                    |                               |                  |                                          |                       |     | CN <sup>-</sup> cons, lb/ton ore | Au recovery, pct total Au |
|-------------------|-------------------------------------------------------|-----------------------------------------------------------------------------------------------------------|--------------------|-------------------------------|------------------|------------------------------------------|-----------------------|-----|----------------------------------|---------------------------|
|                   |                                                       | Experimental calculated head, oz Au/ton ore                                                               | Cement, lb/ton ore | Reagents Cyanide, lb/ton soln | Moisture, wt-pct | Percolation rate, gal/hr/ft <sup>2</sup> | Leaching period, days |     |                                  |                           |
| Clayey silver ore | None                                                  | 2.3                                                                                                       | —                  | 1.0                           | —                | 0.1                                      | 22                    | 0.9 | 73.8                             |                           |
| Clayey silver ore | Particle agglomeration with cement + H <sub>2</sub> O | 2.4                                                                                                       | 10                 | 1.0                           | 9.6              | 15.1                                     | 11                    | 0.6 | 75.4                             |                           |
| Clayey silver ore | Particle agglomeration with cement + CN               | 2.3                                                                                                       | 10                 | 12.0*                         | 9.0              | 19.0                                     | 2.3                   | 0.6 | 78.3                             |                           |

\*Based on cyanide content of the pretreatment solution.

resulted in substantially improved percolation rates (19.2 and 21.1 gal/hr/ft<sup>2</sup>, respectively). Moreover, pretreatment with the combination of cement and cyanide solution resulted in substantially reduced leaching time.

Where, however, the feed consisted of the clayey gold ore sample, agglomeration of fines, with the combination of cement and either water or cyanide solution, was essential to achievement of adequate percolation rates (0.5 vs 19.7 and 19.5 gal/hr/ft<sup>2</sup>). Furthermore, required leaching time was substantially reduced, particularly when the combination of cement and cyanide solution was employed in pretreatment.

#### EXAMPLE 2

In this example, an extremely clayey silver ore containing 2.3 oz Ag/ton was employed in leaching experiments. A series of three column leach tests using 50 lbs of ore crushed to a nominal  $\frac{1}{8}$  inch feed size were con-

55  
56  
57  
58  
59  
60  
61  
62  
63  
64  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
770  
771  
772  
773  
774  
775  
776  
777  
778  
779  
780  
781  
782  
783  
784  
785  
786  
787  
788  
789  
780  
781  
782  
783  
784  
785  
786  
787  
788  
789  
790  
791  
792  
793  
794  
795  
796  
797  
798  
799  
790  
791  
792  
793  
794  
795  
796  
797  
798  
799  
800  
801  
802  
803  
804  
805  
806  
807  
808  
809  
800  
801  
802  
803  
804  
805  
806  
807  
808  
809  
810  
811  
812  
813  
814  
815  
816  
817  
818  
819  
810  
811  
812  
813  
814  
815  
816  
817  
818  
819  
820  
821  
822  
823  
824  
825  
826  
827  
828  
829  
820  
821  
822  
823  
824  
825  
826  
827  
828  
829  
830  
831  
832  
833  
834  
835  
836  
837  
838  
839  
830  
831  
832  
833  
834  
835  
836  
837  
838  
839  
840  
841  
842  
843  
844  
845  
846  
847  
848  
849  
840  
841  
842  
843  
844  
845  
846  
847  
848  
849  
850  
851  
852  
853  
854  
855  
856  
857  
858  
859  
850  
851  
852  
853  
854  
855  
856  
857  
858  
859  
860  
861  
862  
863  
864  
865  
866  
867  
868  
869  
860  
861  
862  
863  
864  
865  
866  
867  
868  
869  
870  
871  
872  
873  
874  
875  
876  
877  
878  
879  
870  
871  
872  
873  
874  
875  
876  
877  
878  
879  
880  
881  
882  
883  
884  
885  
886  
887  
888  
889  
880  
881  
882  
883  
884  
885  
886  
887  
888  
889  
890  
891  
892  
893  
894  
895  
896  
897  
898  
899  
890  
891  
892  
893  
894  
895  
896  
897  
898  
899  
900  
901  
902  
903  
904  
905  
906  
907  
908  
909  
900  
901  
902  
903  
904  
905  
906  
907  
908  
909  
910  
911  
912  
913  
914  
915  
916  
917  
918  
919  
910  
911  
912  
913  
914  
915  
916  
917  
918  
919  
920  
921  
922  
923  
924  
925  
926  
927  
928  
929  
920  
921  
922  
923  
924  
925  
926  
927  
928  
929  
930  
931  
932  
933  
934  
935  
936  
937  
938  
939  
930  
931  
932  
933  
934  
935  
936  
937  
938  
939  
940  
941  
942  
943  
944  
945  
946  
947  
948  
949  
940  
941  
942  
943  
944  
945  
946  
947  
948  
949  
950  
951  
952  
953  
954  
955  
956  
957  
958  
959  
950  
951  
952  
953  
954  
955  
956  
957  
958  
959  
960  
961  
962  
963  
964  
965  
966  
967  
968  
969  
960  
961  
962  
963  
964  
965  
966  
967  
968  
969  
970  
971  
972  
973  
974  
975  
976  
977  
978  
979  
970  
971  
972  
973  
974  
975  
976  
977  
978  
979  
980  
981  
982  
983  
984  
985  
986  
987  
988  
989  
980  
981  
982  
983  
984  
985  
986  
987  
988  
989  
990  
991  
992  
993  
994  
995  
996  
997  
998  
999  
990  
991  
992  
993  
994  
995  
996  
997  
998  
999  
1000  
1001  
1002  
1003  
1004  
1005  
1006  
1007  
1008  
1009  
1000  
1001  
1002  
1003  
1004  
1005  
1006  
1007  
1008  
1009  
1010  
1011  
1012  
1013  
1014  
1015  
1016  
1017  
1018  
1019  
1010  
1011  
1012  
1013  
1014  
1015  
1016  
1017  
1018  
1019  
1020  
1021  
1022  
1023  
1024  
1025  
1026  
1027  
1028  
1029  
1020  
1021  
1022  
1023  
1024  
1025  
1026  
1027  
1028  
1029  
1030  
1031  
1032  
1033  
1034  
1035  
1036  
1037  
1038  
1039  
1030  
1031  
1032  
1033  
1034  
1035  
1036  
1037  
1038  
1039  
1040  
1041  
1042  
1043  
1044  
1045  
1046  
1047  
1048  
1049  
1040  
1041  
1042  
1043  
1044  
1045  
1046  
1047  
1048  
1049  
1050  
1051  
1052  
1053  
1054  
1055  
1056  
1057  
1058  
1059  
1050  
1051  
1052  
1053  
1054  
1055  
1056  
1057  
1058  
1059  
1060  
1061  
1062  
1063  
1064  
1065  
1066  
1067  
1068  
1069  
1060  
1061  
1062  
1063  
1064  
1065  
1066  
1067  
1068  
1069  
1070  
1071  
1072  
1073  
1074  
1075  
1076  
1077  
1078  
1079  
1070  
1071  
1072  
1073  
1074  
1075  
1076  
1077  
1078  
1079  
1080  
1081  
1082  
1083  
1084  
1085  
1086  
1087  
1088  
1089  
1080  
1081  
1082  
1083  
1084  
1085  
1086  
1087  
1088  
1089  
1090  
1091  
1092  
1093  
1094  
1095  
1096  
1097  
1098  
1099  
1090  
1091  
1092  
1093  
1094  
1095  
1096  
1097  
1098  
1099  
1100  
1101  
1102  
1103  
1104  
1105  
1106  
1107  
1108  
1109  
1100  
1101  
1102  
1103  
1104  
1105  
1106  
1107  
1108  
1109  
1110  
1111  
1112  
1113  
1114  
1115  
1116  
1117  
1118  
1119  
1110  
1111  
1112  
1113  
1114  
1115  
1116  
1117  
1118  
1119  
1120  
1121  
1122  
1123  
1124  
1125  
1126  
1127  
1128  
1129  
1120  
1121  
1122  
1123  
1124  
1125  
1126  
1127  
1128  
1129  
1130  
1131  
1132  
1133  
1134  
1135  
1136  
1137  
1138  
1139  
1130  
1131  
1132  
1133  
1134  
1135  
1136  
1137  
1138  
1139  
1140  
1141  
1142  
1143  
1144  
1145  
1146  
1147  
1148  
1149  
1140  
1141  
1142  
1143  
1144  
1145  
1146  
1147  
1148  
1149  
1150  
1151  
1152  
1153  
1154  
1155  
1156  
1157  
1158  
1159  
1150  
1151  
1152  
1153  
1154  
1155  
1156  
1157  
1158  
1159  
1160  
1161  
1162  
1163  
1164  
1165  
1166  
1167  
1168  
1169  
1160  
1161  
1162  
1163  
1164  
1165  
1166  
1167  
1168  
1169  
1170  
1171  
1172  
1173  
1174  
1175  
1176  
1177  
1178  
1179  
1170  
1171  
1172  
1173  
1174  
1175  
1176  
1177  
1178  
1179  
1180  
1181  
1182  
1183  
1184  
1185  
1186  
1187  
1188  
1189  
1180  
1181  
1182  
1183

- substantial reaction of the cyanide with gold or silver values in the feed, and
- (4) subjecting the aged admixture to percolation leaching with water or cyanide solution, whereby gold or silver is selectively leached.
2. The process of claim 1 in which the feed material is a low-grade clayey gold or silver ore, tailing or waste.
3. The process of claim 2 in which the binding agent is portland cement.

4. The process of claim 1 in which the aging time is about 5 to 72 hours.
5. The process of claim 1 in which the aqueous cyanide solution consists of a 1.16 to 1.27 molar solution of sodium cyanide.
6. The process of claim 1 in which the percolation leaching consists of heap leaching.
7. The process of claim 1 in which the percolation leaching consists of vat or flood leaching.

\* \* \* \* \*